

Aug. 24, 1948.

P. D. WILLIAMS

2,447,973

COATED ANODE FOR ELECTRON DISCHARGE DEVICES

Original Filed April 6, 1946



INVENTOR  
*Paul D. Williams*  
BY *Harold E. Eng*

ATTORNEY

## UNITED STATES PATENT OFFICE

2,447,973

COATED ANODE FOR ELECTRON  
DISCHARGE DEVICES

Paul D. Williams, Palo Alto, Calif., assignor to  
Eitel-McCullough, Inc., San Bruno, Calif., a  
corporation of California

Original application April 6, 1946, Serial No.  
660,263. Divided and this application April 21,  
1947, Serial No. 742,773

1 Claim. (Cl. 250—27.5)

2

This is a division of my copending application  
Serial No. 660,263, filed April 6, 1946.

My invention relates to electrodes for elec-  
tron tubes.

It is among the objects of my invention to  
improve the heat dissipation and gettering prop-  
erties of electrodes such as anodes.

Another object is to provide an electrode hav-  
ing a surface layer which is stable at high tem-  
peratures.

The invention possesses other objects and fea-  
tures of advantage, some of which, with the fore-  
going, will be set forth in the following descrip-  
tion of my invention. It is to be understood that  
I do not limit myself to this disclosure of species  
of my invention as I may adopt variant embodi-  
ments thereof within the scope of the claim.

Referring to the drawing:

The figure of the drawing is an elevational  
view of a tube embodying my improvements.

In terms of broad inclusion, my electrode for  
an electron tube comprises a surface layer of me-  
tallic particles bonded together and to the elec-  
trode. The particles making up the surface  
layer include carbon and a metal such as zir-  
conium, tantalum or molybdenum, zirconium being  
preferred, the carbon being combined with  
the metal to form a metallic carbide. In the  
case of an anode the improved electrode prefer-  
ably comprises a hollow body of sheet metal, such  
as molybdenum, upon the outer surface of which  
the carbide layer is applied. The surface layer  
is preferably formed by coating the electrode  
with a mixture of finely divided metal and car-  
bon, the major proportion of which is metal, and  
then heating the electrode to convert the car-  
bon to the carbide and sinter the particles to-  
gether and to the electrode.

In greater detail, and referring to the drawing,  
a tube illustrating my improvements comprises  
an envelope 2 having a reentrant stem 3 carrying  
an exhaust tubulation 4. A base 6 with  
prongs 7 is provided at the lower end of the tube.  
The envelope encloses a cathode 8, grid 11 and  
tubular anode 9, the anode having a cap 12 sup-  
ported by bracket 13 on a lead 14 sealed to the  
upper portion of the envelope.

Grid 11 is of the cage type having a base ring  
21 supported by brackets 22 on rods 23, one of  
which serves as a grid lead connected to a base  
prong 7 by a conductor 24. Cathode 8 is of the  
filamentary type comprising a spiral of thori-  
ated tungsten wire welded top and bottom to a  
pair of leads 17 sealed to stem 3 and connected  
to a pair of base prongs by conductors 18.

The above described tube structure is merely  
for purposes of illustration and may be varied  
within wide limits.

My improvements, as embodied in anode 9,  
comprise a surface layer 15 of carburized me-  
tallic particles bonded or sintered together and  
to the anode body. Body 9 is of a suitable refrac-  
tory metal having a high melting point and low  
vapor pressure, molybdenum being preferred be-  
cause it can be fabricated in sheet form and is  
relatively cheap compared to other metals in  
this class.

The particles in surface layer 15 comprise car-  
bon combined as a carbide with a refractory  
metal or a combination of refractory metals,  
such as zirconium, tantalum, molybdenum or  
tungsten, zirconium being the preferred metal  
for several reasons hereinafter recited. The sur-  
face layer is preferably formed by preparing a  
fluid mixture of the finely divided metal and  
carbon, and applying this mixture to the elec-  
trode by brushing or spraying. In the case of a  
coating containing molybdenum, for example,  
the proportions are preferably 80 parts by weight  
of molybdenum powder to 10 parts of carbon  
powder, it being noted that the major propor-  
tion of the mixture is of the metal. In the case  
of a coating containing zirconium the ratio is  
preferably 91.2 parts by weight of zirconium pow-  
der to 6 parts carbon. These proportions provide  
about half the theoretical amount of carbon re-  
quired to convert all of the metal in the coating  
to the carbide. In either case the powders are  
mixed with a suitable vehicle such as amyl ace-  
tate to a consistency for brushing or spraying.

After coating, the electrode is heated to a tem-  
perature sufficient to convert the carbon to a  
carbide and to sinter the particles together and  
to the electrode body. This heating is carried  
out in an oxygen free atmosphere such as in  
vacuum or in an inert gas such as argon or helium.  
Heating in vacuum is preferred because the  
coating is outgassed simultaneously with the  
carburizing step. With a coating containing  
molybdenum powder I have secured the desired  
result by firing the electrode in a vacuum fur-  
nace to about 1800° C. for about 5 minutes. With  
the preferred coating containing zirconium pow-  
der the firing is preferably done at a lower tem-  
perature for a longer period, say at 1400° C. for  
about 30 minutes. After firing, the anode struc-  
ture is ready for sealing into the envelope, the  
tube from this point on being processed and  
evacuated in the usual manner.

My coated electrode has several advantages.

One is that the final layer, being formed with metallic carbide particles, is of a rough granular texture in addition to being quite dark in color. This black body effect gives the electrode excellent heat dissipation properties. Another feature is that the metallic carbide layer is very stable at high temperatures, which stability is important during processing the tube on the pump and during subsequent operation. The fact that an excess of metal is provided in the coating, over and above that required to satisfy the carbon, means that the final coating contains some pure metal along with the metallic carbide, so that the surface layer 15 comprises an intimate admixture of metal carbide and uncombined metal. Some of the pure metal is probably present as uncombined metal in the core parts of the metallic carbide particles and some probably as metal particles between the carbide particles. In any event, the presence of this uncombined metal aids in binding the metallic carbide together in the coating, resulting in a very tightly cemented layer after the sintering operation. Such a firmly bonded layer is important to prevent the particles from being dislodged under the electrical and thermal stresses set up in the tube during operation.

While any of the metals mentioned in connec-

tion with the coating composition will yield the above mentioned desirable characteristics in the surface layer, I prefer to use zirconium powder because it has additional advantages. For example, a layer composed of zirconium and carbon has good gettering (gas absorption) properties for cleaning up residual gases in the tube. Also, a surface layer containing zirconium carbide tends to suppress electron emission from the electrode. Both of these characteristics are desirable in an anode.

I claim:

An anode for an electron tube, comprising a metallic body, and a surface layer comprising an intimate admixture of zirconium carbide and uncombined zirconium bonded together and to the anode body.

PAUL D. WILLIAMS.

#### REFERENCES CITED

The following references are of record in the file of this patent:

#### UNITED STATES PATENTS

| 25. Number | Name       | Date          |
|------------|------------|---------------|
| 2,232,083  | Strohfeldt | Feb. 18, 1941 |
| 2,368,060  | Wooten     | Jan. 23, 1945 |